

## UNITED STATES PATENT OFFICE

2,652,368

## LUBRICATING OIL COMPOSITION

Donald S. Melstrom and Forrest J. Watson, Oakland, Calif., assignors to Shell Development Company, San Francisco, Calif., a corporation of Delaware

No Drawing. Application June 21, 1949,  
Serial No. 100,544

11 Claims. (Cl. 252—48.2)

1

This invention relates to lubricating oil compositions having improved viscosity characteristics. It is concerned particularly with lubricants containing polymers of alkylene sulfones and their use in improving the temperature viscosity relationship of lubricating oils.

Of the many properties of a lubricating oil considered in commercial evaluation, viscosity is particularly stressed as being significant together with the susceptibility of viscosity to temperature changes. Such an evaluation is usually made with reference to the viscosity index scale advanced by Dean and Davis. The viscosity index figures which follow hereinafter refer to this scale which is well known in the art. According to this scale, the viscosity of an oil is determined at 100° F. and 210° F. in Saybolt Universal seconds. If an oil has a low viscosity index, the viscosity changes rapidly with temperature while a high viscosity index indicates relative insensitivity to thermal influences.

The addition of extraneous compounds to lubricating oils to improve their viscosity temperature relationship is a well developed art. A number of polymeric compounds of simple hydrocarbons have been utilized for this purpose, such as polyisobutylene. A second type of polymeric material found to be of use for improvement in viscosity index includes polymers of esterified methacrylic acid. While each of these types of materials is effective to a certain extent, they exhibit shortcomings which appear to be inherent in their chemical structure. The isobutylene polymers, for example, are subject to depolymerization when an oil containing them is used for a period of time at high engine operating temperatures. It appears that differences in molecular structure are a determining feature in the relative solubility, effectiveness and stability as a viscosity improving agent in lubricating oils.

It is an object of the present invention to provide improved lubricating compositions. It is a further object of this invention to provide lubricating compositions having improved viscosity temperature relationships. It is a special object of this invention to provide lubricating compositions particularly suitable for use in friction drive torque converters. Other objects will become apparent hereinafter.

Now, in accordance with this invention, it has been found that polymeric alkylene sulfones have exceptional properties for improving the viscosity and viscosity index of lubricants. Still in accordance with this invention, it has been discovered that the polymeric alkylene sulfones having from

2 to 4 carbon atoms between sulfone groups and having an alkyl side chain of 5 to 16 carbon atoms directly attached to one of the carbon atoms separating the sulfone groups are especially desirable because of a particularly unique modified dilatancy in mineral oils. Again in accordance with the present invention, the latter polymeric sulfones when compounded with mineral lubricating oils are particularly useful as the lubricant in friction gear torque converters.

The polymeric sulfones with which the present invention is concerned may be prepared by several alternative methods. Polymeric alkylene sulfones having 2 or 4 carbon atoms between sulfone groups are readily prepared by action of sulfur dioxide at low temperatures on monoolefins or conjugated diolefins. A general description of the preparation of typical sulfones included in this group is to be found in a paper by R. D. Snow and F. E. Frey, Journal of Industrial and Engineering Chemistry, vol. 30, 1938, pages 176-182. A second variety of polymeric alkylene sulfone is that containing at least 5 carbon atoms between the sulfone groups. Materials of this description are disclosed in United States Patent 2,201,884 to W. H. Carothers. Sulfones of this latter group are prepared by oxidation of polymeric alkylene sulfides. A particularly desirable group of polymers for use in the present invention comprises the copolymers of sulfur dioxide with alpha-olefinic hydrocarbons having from 7 to 24 carbon atoms. Olefins derived from the cracking of paraffin wax, referred to as "cracked wax olefins" may be used in the preparation of the subject polymers. These include, for example, the alpha varieties of heptene, decene, dodecene, tetradecene and octadecene, including both normal and branched-chain isomers. Copolymerization of this type of alpha-olefin with sulfur dioxide results in the formation of high molecular weight polymeric materials having 2 carbon atoms between sulfone groups, one of the carbon atoms having an alkyl substituent which preferably may vary between 5 and 16 carbon atoms in length. The reason for this preference in structure lies in the fact that polymers of this variety exhibit an unusual variety of dilatancy when dispersed in mineral lubricating oils. An ordinary dilatant fluid is one which thickens when subjected to shear and which immediately regains its normal fluidity when the shearing force is removed. In the present instance, it has been found that mineral oils containing polyalkylene sulfones of the above preferred description exhibit increased thickening when subjected to agitation or stirring

and that upon cessation of this stress, the composition only gradually returns to its original state of fluidity. This peculiar property makes these compositions especially useful in friction drive torque converters.

One of the limiting features of friction gears and similar mechanisms up to the present time has been the unsatisfactory performance of lubricants or fluids used with them for their lubrication and prevention of wear. In the act of lubricating or preventing wear, a film of oil between the friction gear surfaces usually results in increased slippage between the contact points of the surfaces of the engaging gears. Hence, the dilatant properties of the present compositions find ready application in the lubrication of friction gears. When force is applied to the gears lubricated with these compositions, the gelling action which results materially reduces the slippage to which ordinary lubricants are subjected.

Another property which makes these new compositions especially useful for friction gear lubrication is the mild extreme pressure characteristics which appear to be due to the presence of the sulfone groups in the polymeric additives. It has been found that lubricating compositions containing small percentages of polymeric alkylene sulfones have maximum seizure load ratings approximately 30% greater than the unmodified lubricating oils. This property adds to the value of the compositions, especially in their use as torque converter fluids.

The lubricants in which the polyalkylene sulfones may be employed include especially mineral lubricating oils and also esters of dicarboxylic acids, such as bis(2-ethylhexyl) sebacate. Another general class of synthetic lubricant useful as base lubricant in compositions of this invention comprises alkylene oxide polymers which may be prepared from alkylene epoxides or alkylene glycols. A particularly useful variety of this type includes the polymers of trimethylene glycol or of propylene oxide. Other well known

sulfones are present in an amount between 0.5% and 5.0%, by weight, based on the weight of the lubricating oil. Other ingredients may be present in the composition such as standard anti-oxidants, extreme pressure additives, additional viscosity index improvers, anti-corrosion agents, and similar materials all as well known in the art. Greases may be prepared containing the polymeric alkylene sulfones and containing the well known grease-forming soaps or the more recently developed inorganic gel greases prepared by the use of silica gel, alumina gel and gels of other inorganic polyvalent metal oxides.

The preferred process as referred to above for the preparation of sulfones useful in the present compositions comprises addition of alpha-olefins to an excess of liquid sulfur dioxide at reflux temperature (-10° C.) in the presence of a catalyst such as peroxides or nitrates. The reaction mixture is stirred at reflux for approximately one-half hour in the presence or absence of inert diluents such as dioxane and the like. The reaction mixture is then permitted to warm to room temperature so as to evaporate unreacted materials. In the case of a higher molecular weight alpha-olefin such as octadecene-1, the reaction may be conducted under pressure at room temperature so as to permit liquefaction of the hydrocarbon. It has been noted that the polymerization reaction proceeds at a negligibly slow rate if either of the reactants is solid. On the other hand, no polymerization appears to occur when the reactants are in a vaporized condition. With these two limitations in mind, a variety of temperatures and pressures may be chosen to maintain the reactants in a liquefied state with a minimum vapor phase present. Ordinarily, this will mean that the temperatures will be between about -20° C. and +30° C., although these temperatures may be increased in either direction with corresponding change in pressure. The following table illustrates conditions under which representative polymeric sulfones of normal olefins may be prepared.

| Olefinic Compound | Moles of Olefinic Compound | Liquid SO <sub>2</sub> , cc. | Additional Solvent | Catalyst or Inhibitor              | Polymer Conv., Percent | Analysis of Polymer |           |           |                                                              |           |           |
|-------------------|----------------------------|------------------------------|--------------------|------------------------------------|------------------------|---------------------|-----------|-----------|--------------------------------------------------------------|-----------|-----------|
|                   |                            |                              |                    |                                    |                        | Found               |           |           | Theory for (C <sub>n</sub> H <sub>2n</sub> SO <sub>2</sub> ) |           |           |
|                   |                            |                              |                    |                                    |                        | Percent C           | Percent H | Percent S | Percent O                                                    | Percent H | Percent S |
| 1-Tetradecene     | 0.25                       | 300                          | dioxane, 0.25 mol. | Peroxide, 0.5 g. TNB               | 92                     | 63.98               | 10.82     | 11.3      | 64.57                                                        | 10.84     | 12.3      |
| 1-Dodecene        | 0.25                       | 250                          | dioxane, 0.45 mol. | 1 g. LiNO <sub>3</sub> in alcohol. | 79                     | 62.22               | 10.42     | 13.3      | 62.01                                                        | 10.41     | 13.8      |
| 1-Decene          | 0.5                        | 250                          | dioxane, 0.25 mol. | do                                 | 86                     | 58.09               | 9.95      | 15.4      | 58.79                                                        | 9.87      | 15.7      |
| 1-Heptene         | 0.5                        | 250                          | do                 | Peroxide, 2 cc. sat. alc.          | 88                     | 50.99               | 8.61      | 19.5      | 51.82                                                        | 8.70      | 19.8      |
| 1-Octadecene      | 0.06                       | b 20                         | none               | NH <sub>4</sub> NO <sub>3</sub> .  | 94                     | 69.36               | 11.67     | 9.05      | 68.80                                                        | 11.47     | 10.1      |

\*TNB is 1,3,5-trinitrobenzene, an inhibitor.

<sup>b</sup>Reaction was carried out in a sealed tube at room temperature.

synthetic and natural lubricants may be used in the present compositions, such as vegetable oils such as castor oil, fish and animal oils, organic phosphates and chlorinated hydrocarbons exemplified by hexachlorobutadiene and tricresyl phosphate. Mixed phosphates or alkyl phosphates may be used as well, such as diphenyl octyl phosphate, trioctyl phosphate or tributyl phosphate.

In order to be effective for the improvement in viscosity index, the polymeric alkylene sulfones should be present in an amount from about 0.1% to about 10.0% by weight. Preferably, the

Due to the insolubility of the polymeric alkylene sulfones in the solvents normally employed for molecular weight determinations, there has been no accurate method developed for estimating the chain length of the polymers described above. Evidence indicates, however, that the polymers have molecular weights generally ranging between about 5,000 and 100,000. Due to the extremely high molecular weights of these substances, the identity of end groups of the linear polymers are substantially immaterial, particularly as to their utility in the present invention. Up to the present time, no anal-

yses of the end group structures have been made. It is believed that at least one of the end groups is in the form of a sulfone group or of a hydroxyl, but neither of these proposals has been firmly established.

In order to illustrate the effect of adding a sulfone to a lubricating oil, the following comparison was made: A given mineral lubricating oil was found to have a viscosity index of 53, with a viscosity at 100° F. of 10.6 centistokes and 2.5 centistokes at 210° F. Upon the addition of 1% by weight of a polymeric octadecene sulfone produced by copolymerization of sulfur dioxide and octadecene-1 at room temperature under pressure, the viscosity index increased to 135, the composition having a viscosity of 18.5 centistokes at 100° F. and 4.0 centistokes at 210° F.

When a mineral lubricating oil is modified by the addition of 0.75% of a polymeric tetradecene sulfone, prepared from tetradecene-1 as described in the above table, the viscosity index is raised from 50 to 96. The addition of 1.5% of a polymeric octene-1 sulfone to the same mineral oil gives a composition having a viscosity index of 116.

The claimed invention is:

1. A lubricant comprising a hydrocarbon lubricating oil base and in admixture therewith a minor amount sufficient to improve the viscosity index of the oil of a copolymer of cracked wax olefins and sulfur dioxide having a molecular weight between about 5000 and 100,000.

2. A lubricating composition comprising a lubricating oil base and in admixture therewith a minor amount sufficient to improve the viscosity index of the oil of a polyalkylene polysulfone each sulfone group being separated by at least 5 carbon atoms, said polysulfone being prepared by oxidation of polymeric alkylene sulfides.

3. A lubricant comprising a hydrocarbon lubricating oil base and in admixture therewith a minor amount sufficient to improve the viscosity index of the oil of a copolymer of cracked wax alpha olefins and sulfur dioxide.

4. A lubricant comprising a hydrocarbon lubricating oil base and in admixture therewith a minor amount sufficient to improve the viscosity index of the oil of a copolymer of cracked wax alpha monoolefins and sulfur dioxide.

5. A lubricating composition comprising a lubricating oil base and in admixture therewith from 0.1% to 10% by weight of a polyalkylene polysulfone prepared from olefins having from 7 to 24 carbon atoms per molecule and said polysulfone being prepared by polymerization of alpha-olefins and sulfur dioxide.

6. A lubricating composition comprising a lubricating oil base and in admixture therewith a minor amount sufficient to improve the viscosity index of the oil of a polyalkylene polysulfone having a molecular weight from about 5,000 to about 100,000 prepared from olefins having from 7 to 24 carbon atoms per molecule said polysulfone being prepared by copolymerization of alpha olefins and sulfur dioxide.

10. 7. A lubricating oil composition exhibiting improved dilatancy comprising a major amount of a mineral lubricating oil base and 0.1 to 10% by weight of a poly(alkylene-1,2 sulfone) having a molecular weight between 5,000 and 100,000, the sulfone groups of which are separated by 2 to 4 carbon atoms, one of which bears an alkyl substituent of 5 to 16 carbon atoms said sulfone being prepared by copolymerization of alpha olefins and sulfur dioxide.

20. 8. A lubricant comprising a hydrocarbon lubricating oil base and in admixture therein a minor amount sufficient to improve the viscosity index of a polysulfone prepared by the polymerization of n-octadecene-1 and SO<sub>2</sub>.

25. 9. A lubricant comprising a hydrocarbon lubricating oil base and in admixture therewith a minor amount sufficient to improve the viscosity index of the oil of a polysulfone prepared by the polymerization of a normal 1-alkene having from 12 to 20 carbon atoms and SO<sub>2</sub>.

30. 10. The process for the lubricating of metallic surfaces which comprises maintaining thereon a lubricating oil composition comprising a hydrocarbon lubricating oil base in admixture therewith a minor amount sufficient to improve the viscosity index of the oil of a polysulfone prepared by the polymerization of a normal 1-alkene having from 12-20 carbon atoms and sulfur dioxide.

35. 11. A lubricant comprising a hydrocarbon lubricating oil base and in admixture therewith a minor amount sufficient to improve the viscosity index of the oil of a copolymer of octene-1 and sulfur dioxide, said copolymer having a molecular weight between about 5,000 and 100,000.

DONALD S. MELSTROM.  
FORREST J. WATSON.

References Cited in the file of this patent

UNITED STATES PATENTS

| Number       | Name          | Date          |
|--------------|---------------|---------------|
| 1,452,946    | Weiss         | Apr. 24, 1923 |
| 2,201,884    | Carothers     | May 21, 1940  |
| 2,225,266    | Frey          | Dec. 17, 1940 |
| 55 2,483,499 | Lieber et al. | Oct. 4, 1949  |